

# UNITED STATES PATENT OFFICE.

ALBERT EDWARD GESSLER, OF CLIFTON, NEW YORK.

## MANUFACTURE OF CHROMIUM OXID.

1,158,379.

Specification of Letters Patent.

Patented Oct. 26, 1915.

No Drawing.

Application filed February 13, 1913. Serial No. 748,153.

*To all whom it may concern:*

Be it known that I, ALBERT EDWARD GESSLER, a citizen of the German Empire, residing at Clifton, in the county of Richmond 5 and State of New York, have invented new and useful Improvements in the Manufacture of Chromium Oxid, of which the following is a specification.

My invention relates to the production of 10 green oxid of chromium from chromates without the employment of external heat and consists generally in the ignition of a proper mixture of a chromate, a reducing agent and a highly oxidizing agent.

15 The present known methods of producing green oxid of chromium from chromates consist in introducing a mixture of the chromate and a reducing agent into a furnace and heating to a high temperature, generally 20 from 500° C. to 700° C., the heat being necessarily obtained from an external source. I have found that a great saving in time, fuel and apparatus can be obtained by adding 25 to the mixture of chromate and reducing agent a quantity of a highly oxidizing agent which will increase the chemical energy of the mixture and allow the formation of oxid of chromium by mere ignition and self combustion of the mixture.

30 In following my process, the chromates I preferably employ are the alkali metal bichromates, for example sodium bichromate and potassium bichromate, the reducing agents being preferably sulfur, carbon or 35 aluminum, and the highly oxidizing agents being preferably alkali metal chlorates, for example sodium chlorate, potassium chlorate and peroxids.

40 The following is an example of one method of performing my invention. Fifty-three hundred (5300) parts of powdered calcined sodium bichromate, one thousand (1000) parts of sulfur flour, and one hundred and twenty-five (125) parts of powdered sodium chlorate are thoroughly mixed together and placed in a proper receptacle. The mixture is then ignited by means of a direct flame and allowed to burn through self combustion. When the combustion has 45 been completed and the mixture converted into a dark green bulky mass, it is allowed

to cool and is thoroughly washed to remove the soluble by-products, and dried if desired. The resulting product is practically pure green oxid of chromium. 55

The fifty three hundred (5300) parts of powdered calcined sodium bichromate may be substituted by fifty-nine hundred (5900) parts of powdered calcined potassium bichromate, the remainder of the process being 60 practically the same.

I do not limit myself to the proportions or particular chemicals mentioned herein, all of which may be varied without going beyond the scope of my invention which comprises the production of green oxid of chromium through the ignition and self combustion of a mixture of a suitable chromate, reducing agent and highly oxidizing agent. 65

Having described my invention, what I 70 claim is:

1. The process of producing green oxid of chromium which comprises making a mixture of an alkali-metal chromate, a reducing agent capable of reducing the chromate to 75 chromium oxid, and an oxidizing agent capable of sustaining combustion, igniting the mixture within a receptacle, allowing the combustion to proceed to the formation of chromium oxid, and lixiviating the resultant 80 product.

2. The process of producing green oxid of chromium which comprises making a mixture of an alkali-metal bichromate, a reducing agent capable of reducing the bichromate 85 to chromium oxid, and an oxidizing agent capable of sustaining combustion, igniting the mixture within a receptacle, allowing the combustion to proceed to the formation of chromium oxid, and lixiviating the resultant 90 product.

3. The process of producing green oxid of chromium which comprises making a mixture of an alkali-metal bichromate, sulfur, and an oxidizing agent capable of sustaining 95 combustion, igniting the mixture within a receptacle, allowing the combustion to proceed to the formation of chromium oxid, and lixiviating the resultant product.

4. The process of producing green oxid of 100 chromium which comprises the ignition and self combustion of a mixture of an alkali

metal bichromate, sulfur and an alkali metal chlorate.

5. The process of producing green oxid of chromium which comprises mixing sodium bichromate, sulfur and sodium chlorate, igniting the mixture, allowing the completion of the combustion, and lixiviating.

In testimony whereof I have signed my name to this specification in the presence of two subscribing witnesses.

ALBERT EDWARD GESSLER.

Witnesses:

CHAS. POPP,  
H. SCHOEFFLER.